# EUROPEAN PATENT SPECIFICATION

(11) **EP 0 924 344 B1**
(45) Date of publication and mention of the grant of the patent: **25.02.2004**
(21) Application number: 98204321.8
(22) Date of filing: 17.12.1998
(51) Int. Cl.: E01B 1/00, E01B 19/00, E01C 9/06, E01C 7/32

(54) **Rail track construction**
Schienengleis
Voie ferrée

(30) Priority: 17.12.1997 NL 1007815
(43) Date of publication of application: 23.06.1999
(73) Proprietor: KONINKLIJKE WEGENBOUW STEVIN B.V., NL-3503 RG Utrecht (NL); HEIJMANS WEGEN- EN WATERBOUW B.V., 5240 AJ Rosmalen (NL)
(72) Inventor: Pronk, Cornelis Pieter, 2172 XR Sassenheim (NL); Heerkens, Josephus Cornelis Petrus, 5258 SN Berlicum (NL)
(74) Representative: van Westenbrugge, Andries

(56) References cited:
- DE-A- 4 430 967
- DE-U- 29 611 725
- NL-A- 7 314 861
- NL-C- 36 958

## Description

The invention relates to a method for laying rails in a pavement having a road surface for traffic, wherein the rails are laid in the pavement such that they are sunken with respect to the road surface according to the preamble of claim 1.

European Patent Application EP-A 0 737 778 in the name of the Applicant discloses a rail track construction with which two parallel rails are laid in grooves in a concrete or steel foundation. A layer of sound-absorbent material such as, for example, very open asphalt concrete (VOAC) is applied between and alongside the rails. How the rails are fixed in the grooves is not shown in more detail. Fixing of the rails is problematical since, on the one hand, a high degree of fixation is desired and, on the other hand, a sound-damping effect must also be obtained and the transfer of vibration from the rails to the foundation, which for example is made of concrete, must be restricted. The construction disclosed in EP-A 0 737 778 is not suitable for use in a road surface for traffic, such as, for example, in the case of tram rails laid in the road. NL patent 36958 discloses a method according to the preamble of claim 1. A rail structure comprising rails and cross members is positioned after which the area in between is filled.

One aim of the present invention is therefore to provide a method for laying rails in a pavement with which stable positioning of the rails can take place in a simple and inexpensive manner. A further aim of the present invention is to provide a method for forming a rail construction which is well integrated in the paving construction of the pavement with relatively few transitions so that a level road surface is retained. A further aim of the present invention is to provide a rail construction wherein adequate vibration damping of the rails is obtained, wherein fixing of the position in the long term under static loads is guaranteed and wherein in the event of replacement the rails can be removed relatively easily. To this end the method according to the present invention has the characterising features of claim 1.

When applying the layer of starting material the latter can be rendered plastic and applied simply with the aid of, for example, known asphalt spreading techniques. The voids in the starting material are then filled with a hardening reinforcing medium so that a fixing course is formed which has very high lateral dimensional stability. As a result the rails are accurately fixed and sleepers, tie bars or other fixing means to join the rails to one another can be dispensed with. Furthermore the method according to the present invention saves costs because the major part of the rail construction is formed by the road paving.

It is possible first to lay the rails in the starting material, for example by cutting grooves in the latter when it is applied or by making said grooves subsequently by sawing or milling and then applying the reinforcing medium. However, it is also possible first to form the fixing course by applying a reinforcing medium and then to lay the rails in preformed and hardened grooves.

Preferably the space between the rails and the wall of the grooves is filled with a casting material, such as a casting material based on plastics, optionally with vibration-damping fillers, or a casting material composed of asphalt.

Preferably, the staring material used for the fixing course is very open asphalt concrete (VOAC) having a voids content of at least 20 %, preferably between 25 % and 30 %. It has been found that such a course allows good penetration of the hardening reinforcing medium and that a highly advantageous lateral dimensional stability is obtained by this means. Preferably, the reinforcing medium comprises a cement-based slurry which has good penetration in very open asphalt concrete.

The thickness of the fixing course is preferably between 5 cm and 15 cm and in a preferred embodiment forms the road surface for the traffic. For alignment in the vertical direction a roadbase comprising asphalt granulate cement formed from recycled asphalt concrete with cement (CRAC) and/or asphalt concrete with minerals such as crushed aggregate or chippings (for example RAC) is preferably used. A basecourse of asphalt concrete with minerals (RAC) can be used on top of this foundation and the fixing course applied on top of this. With a construction of this type some flexibility in the vertical direction is retained, as a result of which cracking in the event of slight settlement is counteracted.

With the method according to the present invention transverse forces of various magnitude, such as, for example, transverse forces which arise when taking bends, can be absorbed by varying the thickness of the fixing course. The thickness of the roadbase is partly dependent on the sub-grade conditions and on the volume of traffic.

The invention will be explained in more detail with reference to the single figure, which shows a diagrammatic cross-section of a tram rail construction according to the present invention. The figure shows a tram rail construction 1 having two rails 2, 2'. each of which has been laid in an individual groove 3. The groove 3 has been made in a fixing course 4 according to the present invention which has been formed from very open asphalt concrete with a hardened cement-based reinforcing medium therein. The fixing course 4 forms a road surface 5 for traffic, the rails 2, 2' being laid flush with the road surface 5.

The rails 2. 2' have been fixed in the grooves 3 by means of a plastic casting material 6, which, for example, is formed from a plastic, optionally with vibration-damping fillers. Below the fixing course there is a basecourse 7 formed from bitumen with crushed aggregate or chippings of a standard composition. A roadbase 8 is used below the basecourse 7, which roadbase 8 can have a composition similar to that of the basecourse 7 or can be formed from crushed used asphalt concrete to which about 4 % by wt cement has been added (CRushed Asphalt Cement or CRAC) which has been made up in accordance with generally known guidelines. Using the method according to the present invention rails can be laid in a pavement in a simple manner, without using sleepers, tie bars or other fixing means, such that a rail construction is obtained that is well integrated in the road surface with a minimum of transitions and minimum unevenness. By using the hardening reinforcing medium according to the present invention the rails 2, 2' can be anchored in a stable manner without the use of sleepers or other tie elements between the rails.

## Claims

1. Method for laying rails in a pavement having a road surface for traffic, wherein the rails are laid in the pavement such that they are sunken with respect to the road surface, wherein the rails are laid in a fixing course that has been formed from a porous starting material having a relatively high voids content, which voids are filled with a hardening reinforcing medium, **characterised in that** grooves, in which the rails can be laid, are first made in the starting material of the fixing course, after which the reinforcing medium is applied.

2. Method according to Claim 1, **characterised in that** the fixing course is first formed and **in that** the grooves are made after the reinforcing medium has hardened.

3. Method according to Claim 1 or 2, **characterised in that** after laying the rails in the grooves the space between the rails and the wall of the grooves is filled with a casting material.

4. Method according to Claim 1, 2 or 3, **characterised in that** the reinforcing medium comprises a cement-based slurry.

5. Method according to one of the preceding claims, **characterised in that** the fixing course comprises very open asphalt concrete (VOAC) having a voids content of at least 20%, preferably between 25% and 30%.

6. Method according to one of the preceding claims, **characterised in that** the casting material comprises a setting plastic or asphalt.

7. Method according to one of the preceding claims, **characterised in that** two parallel rails are laid without joining said rails to one another by sleepers.

8. Method according to one of the preceding claims, **characterised in that** the thickness of the fixing course is between 5 cm and 15 cm.

9. Method according to one of the preceding claims, **characterised in that** the fixing course forms the road surface.

10. Method according to one of the preceding claims, **characterised in that** the fixing course is applied on top of a roadbase comprising recycled asphalt concrete with cement (CRAC) and/or asphalt concrete with minerals such as crushed aggregate or chippings (RAC).

11. Method according to Claim 10, **characterised in that** paving of asphalt concrete with minerals such as crushed aggregate or chippings is applied on top of the roadbase.

12. Method according to one of the preceding claims, **characterised in that** the grooves for laying the rails extend partially into the basecourse located beneath the fixing course.

13. Method according to one of the preceding claims, **characterised in that** the rails (2, 2') are not joined to another by tie elements.

## Patentansprüche

1. Verfahren zum Verlegen von Schienen in einen Oberbau mit einer Straßenoberfläche für den Verkehr, wobei die Schienen so in den Oberbau gelegt werden, daß sie bezüglich der Straßenoberfläche versenkt sind, wobei die Schienen in einer Befestigungsschicht verlegt werden, die aus einem porösen Ausgangsmaterial mit einem relativ hohen Porengehalt hergestellt worden ist, wobei die Poren mit einem härtenden Verstärkungsmittel gefüllt werden, **dadurch gekennzeichnet, daß** zuerst Rillen, in welche die Schienen verlegt werden können, in dem Ausgangsmaterial der Befestigungsschicht ausgebildet werden und danach das Verstärkungsmittel angewandt wird.

2. Verfahren nach Anspruch 1, **dadurch gekennzeichnet, daß** zuerst die Befestigungsschicht ausgebildet wird und daß die Rillen ausgebildet werden, nachdem das Verstärkungsmittel ausgehärtet ist.

3. Verfahren nach Anspruch 1 oder 2, **dadurch gekennzeichnet, daß** nach Verlegen der Schienen in den Rillen der Raum zwischen den Schienen und der Wand der Rillen mit einem Gußmaterial gefüllt wird.

4. Verfahren nach Anspruch 1, 2 oder 3, **dadurch gekennzeichnet, daß** das Verstärkungsmittel einen Schlamm auf Zementbasis aufweist.

5. Verfahren nach einem der vorstehenden Ansprüche, **dadurch gekennzeichnet, daß** die Befestigungsschicht einen sehr offenen Asphaltbeton (VOAC) aufweist, der einen Porengehalt von mindestens 20%, vorzugsweise zwischen 25% und 30%, hat.

6. Verfahren nach einem der vorstehenden Ansprüche, **dadurch gekennzeichnet, daß** das Gußmaterial einen abbindenden Kunststoff oder Asphalt aufweist.

7. Verfahren nach einem der vorstehenden Ansprüche, **dadurch gekennzeichnet, daß** zwei parallele Schienen verlegt werden, ohne die Schienen durch Schwellen miteinander zu verbinden.

8. Verfahren nach einem der vorstehenden Ansprüche, **dadurch gekennzeichnet, daß** die Dicke der Befestigungsschicht zwischen 5 cm und 15 cm ist.

9. Verfahren nach einem der vorstehenden Ansprüche, **dadurch gekennzeichnet, daß** die Befestigungsschicht die Straßenoberfläche bildet.

10. Verfahren nach einem der vorstehenden Ansprüche, **dadurch gekennzeichnet, daß** die Befestigungsschicht auf einen Unterbau aufgebracht wird, der wiederverwerteten Asphaltbeton mit Zement (CRAC) und/oder Asphaltbeton mit Mineralen, beispielsweise zerkleinertem Granulat oder Splitt (RAC) aufweist.

11. Verfahren nach Anspruch 10, **dadurch gekennzeichnet, daß** Belag aus Asphaltbeton mit Mineralen, beispielsweise zerkleinertem Granulat oder Splitt, auf den Unterbau aufgebracht wird.

12. Verfahren nach einem der vorstehenden Ansprüche, **dadurch gekennzeichnet, daß** die Rillen zum Verlegen der Schienen sich teilweise in die Basisschicht erstrecken, die sich unterhalb der Befestigungsschicht befindet.

13. Verfahren nach einem der vorstehenden Ansprüche, **dadurch gekennzeichnet, daß** die Schienen (2,2') nicht durch Verbindungselemente miteinander verbunden sind.

## Revendications

1. Procédé pour disposer des rails dans une chaussée comportant une surface de roulement pour le trafic, dans lequel les rails sont disposés dans la chaussée de telle sorte qu'ils soient en contrebas par rapport à la surface de roulement dans lequel les rails sont disposés dans une couche de fixation qui a été réalisée en un matériau de départ poreux ayant une teneur en vides relativement élevée, lesquels vides sont remplis d'un milieu de renforcement durcissant, **caractérisé en ce que** des rainures, dans lesquels les rails peuvent être disposés, sont d'abord réalisées dans le matériau de départ de la couche de fixation, après quoi le milieu de renforcement est appliqué.

2. Procédé selon la revendication 1, **caractérisé en ce que** la couche de fixation est d'abord formée et **en ce que** les rainures sont réalisées après le durcissement du milieu de renforcement.

3. Procédé selon la revendication 1 ou 2, **caractérisé en ce que**, après avoir disposé les rails dans les rainures, l'espace compris entre les rails et la paroi des rainures est rempli d'un matériau de coulée.

4. Procédé selon la revendication 1, 2 ou 3, **caractérisé en ce que** le milieu de renforcement comprend une suspension à base de ciment.

5. Procédé selon l'une des revendications précédentes, **caractérisé en ce que** la couche de fixation comprend du béton bitumineux à enrobés très ouverts (VOAC) ayant une teneur en vides d'au moins 20 %, de préférence comprise entre 25 % et 30 %.

6. Procédé selon l'une des revendications précédentes, **caractérisé en ce que** le matériau de coulée comprend un plastique durcissable ou de l'asphalte.

7. Procédé selon l'une des revendications précédentes, **caractérisé en ce que** deux rails parallèles sont disposés sans relier lesdits rails l'un à l'autre par des traverses.

8. Procédé selon l'une des revendications précédentes, **caractérisé en ce que** l'épaisseur de la couche de fixation est comprise entre 5 cm et 15 cm.

9. Procédé selon l'une des revendications précédentes, **caractérisé en ce que** la couche de fixation forme la surface de roulement.

10. Procédé selon l'une des revendications précédentes, **caractérisé en ce que** la couche de fixation est appliquée sur une couche de base comprenant du béton bitumineux recyclé avec du ciment (CRAC) et/ou du béton bitumineux avec des minéraux tels qu'un agrégat concassé ou des gravillons (RAC).

11. Procédé selon la revendication 10, **caractérisé en ce que** le revêtement de béton bitumineux avec des minéraux tels qu'un agrégat concassé ou des gravillons est appliqué sur la couche de base.

12. Procédé selon l'une des revendications précédentes, **caractérisé en ce que** les rainures pour disposer les rails s'étendent partiellement dans la couche de base située au-dessous de la couche de fixation.

13. Procédé selon l'une des revendications précédentes, **caractérisé en ce que** les rails (2, 2') ne sont pas reliés l'un à l'autre par des éléments d'ancrage.
